

May 28, 1940.

T. REICHERT

2,202,231

PROCESS FOR THE CARBONIZATION OF WOOD AND SIMILAR MATERIALS

Filed March 11, 1938

*Fig. 1.*



*Fig. 2.*



Inventor  
THEOPHIL REICHERT,

By *Bailey & Parsons*  
Attorney

## UNITED STATES PATENT OFFICE

2,202,231

PROCESS FOR THE CARBONIZATION OF  
WOOD AND SIMILAR MATERIALS

Theophil Reichert, Brilon Wald, Germany, assignor, by mesne assignments, to Chemical Marketing Company Inc., New York, N. Y.

Application March 11, 1938, Serial No. 195,415  
In Germany March 13, 1937

3 Claims. (Cl. 202—15)

The invention relates to a process for the carbonization of wood and similar materials. It especially relates to that type of carbonization in which all of the heat is supplied to the wood by heating gases, and no other heating of the wood is provided.

Such procedures have presented certain difficulties since the large amounts of gas used make it difficult to condense or wash out the distillation products. Where attempts have been made to reduce the amount of gas, overheating and a reduction in yield have generally resulted.

The present invention provides a manner of carbonizing wood so as to obtain high yields while utilizing a relatively small amount of circulating gases so that it is easy to recover the distillation products of the wood.

Suitable retorts for use in the process herein disclosed are shown in the drawing. Fig. 1 shows a retort with an inclination of 60° for the upper wall and 40° for the lower wall. Fig. 2 shows 55° for the upper wall and 45° for the lower wall.

In order to carry out the process, it has been found that the most important feature is the linear speed of movement of the circulating gas as it passes through the wood, and by suitable regulation of this linear speed improved results may be obtained regardless of the volume of carbonization gas per unit of wood passing through the retort. By suitable adjustment of the linear speed we have found it possible to carry out the carbonization under the best conditions, regardless of the moisture content of the wood. For this purpose it is important that the linear speed should lie within a certain range.

In the ordinary carbonization of wood by heated circulating gases the temperature in the carbonization zone, which gradually moves downwardly through the mass of wood during the carbonization process, is higher than the temperature of the previously carbonized layers above the carbonization zone. This is true at very low linear speeds of the circulating gases. If the rate of circulation is increased, it will be found that at a certain point the temperature excess of the carbonization layer over the upper layers disappears. When this point is reached, decreases in yield are avoided, and an economical process is thereby possible. In other words, according to the invention it is important that the linear speed of the circulating gases should be high enough to prevent a greater temperature in the carbonization zone than in the zones thereabove.

On the other hand, the use of too high a speed at the ordinary temperature and pressures is

undesirable. This speed should not exceed about 50 cm. per second, and advantageously should not exceed 20 cm. per second.

By maintaining the speed thus within a range of 1 to 50 cm. per second, it is possible to obtain high yields under conditions such that separation of the distillation products is easily possible. Even predried wood can be thus treated with excellent results. In carrying out the operation, all that is necessary is to provide a number of 10 thermometers at different heights in the retort, and to vary the speed of the circulating gases in accordance with the indications of these thermometers so that the temperatures in the upper layers are not less than that in the carbonization zone.

## Example 1

An upright heat-insulated carbonization retort with a capacity of approximately 100 cubic meters was filled with about 40 cubic meters of wood with a moisture content of 22%. Hot gases were introduced at the top of the retort and passed downwardly therethrough, these gases when introduced having a temperature of 450° C. to 500° C. The gases were introduced at a rate of about 2 to 3 cm. per second, and this rate was maintained in such a manner by the observation of thermometers that no temperature differences occurred in the various zones. Carbonization began promptly and was completed without permitting the operation to stop. During the main period of the carbonization distillation products escaped at the lower part of the retort at temperatures between 60 and 150° C. The yield per 35 cubic meter<sup>4</sup> of wood was as follows:

|                   | Kilogram |
|-------------------|----------|
| Acetic acid.....  | 43 to 44 |
| Wood alcohol..... | 14.5     |
| Wood tar.....     | 63.9 40  |
| Charcoal.....     | 200      |

The charcoal was uniformly charred throughout.

Various gases may be used as heating gases, such as combustion gases from furnaces or the like or exhaust gases of internal combustion engines. Also gases produced by the burning of liquid or dust-like fuels may be utilized as heating gases. Preferably the combustible gases obtained from the carbonization are used, partly as circulating gases, while another part of these distillation products are burned for heating the circulating gases. Flushing gases may also be used as a heat carrier if the temperatures of the carbonization material are maintained at least as 55

high as 500° C., and preferably between 550° C. and 750° C.

The operation of the process was not obvious since it was to be expected that the exothermic reaction would occur to an increased degree under such conditions. It was furthermore feared that the surfaces of the pieces being carbonized would be so unfavorably influenced by the strong carbonization reaction that proper carbonization would be impossible. Furthermore, a breaking up of the carbonization material was to be expected which would produce a considerable decrease in the value of the charcoal obtained. Also, and most important, such a process would apparently produce a decrease in the yield of the distillation products which are very sensitive to higher temperature, especially in the presence of a catalytic material such as charcoal. However, according to the invention, none of these results arises, but on the contrary, a high yield is obtained.

Furthermore, since the carbonization can be carried out more quickly the apparatus in which it is carried out may be used oftener. The process is applicable to wood, lignin, peat or other raw materials of vegetable origin.

*Example 2*

A heat-insulated carbonization retort with a capacity of 100 cm. was filled with wood having a moisture content of 20.5%. Carbonization gas from a preceding operation was heated in a superheater and passed downwardly through the material so that it was heated to from 550° C. to 600° C. The linear speed of the heating gases was kept at 1 to 2 cm. per second. The distillation products were freed in condensers from tar, wood, vinegar and the like, and in washing towers from wood alcohol. The combustible gases remaining were partly recirculated, and partly burned for heating the recirculating gases. The yields per cubic meter were as follows:

|              | Kilograms |
|--------------|-----------|
| Acetic acid  | 44 to 45  |
| Wood alcohol | 15        |
| Wood tar     | 63.5      |
| Charcoal     | 200       |

The present process can be carried out continuously, semicontinuously, or periodically. The material to be carbonized may be in large pieces, briquettes, or in the form of dust.

The carbonization procedure is preferably carried out in a retort of special shape. In the past retorts for carbonization have been unsatisfactory for various reasons, one of them being that

these retorts cannot be completely filled so that spaces occur therein which trap the gases and cause improper circulation. This prevents the constant movement of the gas at the desired velocity and thus makes it difficult to maintain the temperature equal in the carbonizing layer and the layers thereabove. According to the present invention such a disadvantage is avoided by making the upper part of the retort in the form of a frustum, for example, a conical frustum, the upwardly converging wall of which forms with the horizontal an angle of at least 50°, and preferably 55° and 65°. Such retorts can be filled uniformly and completely with wood or other carbonization material. As shown in Fig. 1, the top part of the upper section may be in the shape of a frustum of a cone. However, as shown in Fig. 2, this upper part may be also in the form of a curved surface, such as a spherical segment, a paraboloid and the like. Various other shapes may be provided as long as the walls where they meet the vertical walls form the proper angle.

It has also been found that improved results can be obtained in my process if the lower downwardly converging walls of the retort are given a suitable angle, preferably an angle of 40° to 50° with the horizontal. Such a shape makes it possible for the material in the retort to slide out completely when the door in the bottom is opened to permit the removal of the charcoal.

While I have described herein some embodiments of my invention, I wish it to be understood that I do not wish to limit myself thereby except within the scope of the appended claims.

I claim:

1. A process for carbonizing cellulosic material of vegetable origin to produce high yields of acetic acid and alcohol, which comprises filling a retort the upper portion of the walls of which forms an upwardly converging angle of between 50° and 65° with the horizontal with such material, and passing hot oxygen-free gases downwardly through such material at a velocity of below 50 cm. per second, the velocity being so regulated that the temperature in the carbonization zone is not greater than that in the zones thereabove, and the temperature of the material being carbonized being maintained between about 500° C. and 750° C.

2. In a process as claimed in claim 1, the lower walls of said retort forming a downwardly converging angle of from 40° to 50° with the horizontal.

3. A process as claimed in claim 1, in which said velocity does not exceed 20 cm. per second.

THEOPHIL REICHERT.